

# United States Patent [19]

Lavitt

[11] 3,868,282

[45] Feb. 25, 1975

[54] **DOUBLE-BASE PROPELLANT  
CONTAINING A UREIDE AND A  
RESORCYLATE**

|           |        |                    |          |
|-----------|--------|--------------------|----------|
| 3,138,499 | 6/1964 | Camp et al. ....   | 149/98 X |
| 3,228,338 | 1/1966 | McEwan et al. .... | 149/98 X |
| 3,379,010 | 4/1968 | Harvey.....        | 149/98 X |

[75] Inventor: **Joseph W. Lavitt, Succasunna, N.J.**

[73] Assignee: **The United States of America as  
represented by the Secretary of the  
Army, Washington, D.C.**

[22] Filed: **June 7, 1967**

[21] Appl. No.: **645,565**

[52] U.S. Cl..... **149/98, 149/95, 149/92,  
149/102**

[51] Int. Cl..... **C06b 5/04**

[58] Field of Search ..... **149/95, 97, 98, 92, 102**

[56] **References Cited**

UNITED STATES PATENTS

3,032,972 5/1962 Preckel..... 149/98 X

*Primary Examiner*—Stephen J. Lechert, Jr.  
*Attorney, Agent, or Firm*—Robert P. Gibson; Nathan  
Edelberg; Edward F. Costigan

[57]

## ABSTRACT

A double-base propellant of nitrocellulose and nitro-glycerin which contains lead resorcylate for an improved exhaust, comparably higher burning rate and higher operating pressure.

**18 Claims, No Drawings**

## DOUBLE-BASE PROPELLANT CONTAINING A UREIDE AND A RESORCYLATE

This invention relates to smokeless double-base propellants containing nitrocellulose and nitroglycerin.

My patent application for "Improved Nitrocellulose Base Propellants," Ser. No. 394,633, filed 4 Sept. 1964, relates to propellants having reduced smoke and moisture contents in their exhaust. A limitation of the propellants covered by the above basic application exist in the low burning rates and relatively low operating pressure obtained. However, some of the propulsion systems in use today require that the propellant produce a pressure of at least 1,000 pounds per square inch and a burning rate of at least 0.25 inches per second in order to operate properly. These latter requirements are not met by the propellants described in the above cited application.

It is therefore an object of this invention to provide a smokeless double-base propellant containing nitrocellulose and nitroglycerin having a relatively greater burning rate and producing a relatively higher operating pressure than that previously obtained by conventional propellants for use in propulsion systems requiring the same.

Other objects and many attendant advantages of this invention will be readily appreciated as the same become better understood by reference to the following detailed description.

It has now been discovered that if a lead salt of a resorcylate is incorporated in the compositions disclosed in the above cited basic application, propellants may be produced having the exhaust properties, the burning rates, and operating pressures desired for special propulsion systems in use today. More specifically, if a lead salt of a resorcylate is added to the compositions of the basic disclosure in an amount between 0.5 and 10.0%, the propellant thereby produced will have a smokeless exhaust, a burning rate of over 0.3 inches per second and an ideal operating pressure between 1,000 and 2,000 pounds per square inch. The lead resorcylate compounds which may be utilized to this advantage include lead alpha-resorcylate, lead beta-resorcylate, and lead gamma-resorcylate.

The basic compositions to which the lead resorcylate material may be incorporated to advantage include double-base propellants containing nitrocellulose and nitroglycerin. The basic compositions above described preferably include the following range of ingredients in specified amounts, on a weight basis, as follows, viz:

1. About 40 to 60% of nitrocellulose having a nitrogen content between about 10 to 14.2%,
2. About 20 to 34% of a nitrate ester of a polyhydroxy alcohol, preferably glycerol trinitrate,
3. About 5 to 25% of an acetate ester of a polyhydroxy alcohol, preferably glycerol triacetate,
4. About 0.5 to 10% of monoalkali salt of a ureide, preferably monosodium barbiturate or sodium barbital,
5. About 0.5 to 5.0% of a stabilizer such as ethyl centralite or 2-nitrodiphenylamine, and
6. Nitrogen bearing coolants such as oxamide may be added in amounts up to about 25% to obtain required flame temperature and ballistic properties.

The above composition may be manufactured by any of the processes available such as the solventless water slurry processing or the plastisol process, although somewhat better mechanical properties and ballistics

are usually obtained when the solventless water slurry process is employed.

The following examples illustrate the manner of producing the composition including the manner of incorporating the lead resorcylate ingredient in the composition.

### EXAMPLE NO. I

A 30 lb. mix of an improved double-base propellant, 10 hereinafter designated SMU-118, was manufactured by the solventless water slurry process which involved adding 14.49 lbs. of nitrocellulose containing about 12.6% nitrogen to 144.9 lbs. of water at 120°F in a 55 gallon mix can equipped with an air driven mixer. The 15 suspension was mixed for 10 minutes after which 8.01 lbs. of nitroglycerin were added. The mixture was again mixed for 10 minutes and a mixture containing 0.96 lbs. of lead beta-resorcylate and 0.30 lbs. of ethyl centralite in 7.23 lbs. of triacetin was added. The suspension was mixed again for 30 minutes after which it was 20 poured into a suitable cotton duck bag. The water was then removed by centrifuging the bag in a suitable wringer to form a paste which was screened through a  $\frac{1}{4}$  inch by  $\frac{1}{4}$  inch mesh screen and dried until the moisture content was 8-12%. The paste was then blended, 0.30 lbs. of sodium barbiturate being added to the paste during the blending. The paste was then rolled on differential speed rolls at 210°F with a roll gap of 0.025 inch  $\pm$  0.005 inch at roller speeds of 22.5 and 15 rpm 25 to obtain differential speed sheets. These sheets were then rolled on even speed rolls to form even speed sheets at 140°  $\pm$  10°F at a roll speed of 11 rpm and roll gap of 0.035 inch  $\pm$  0.005 inch.

### EXAMPLE NO. II

A 1,700 lb. mix of an improved double base propellant, hereinafter designated SMU-119, was manufactured by the solventless water slurry process which involved adding 821.1 lbs. of nitrocellulose containing about 12.6% nitrogen to 9,853 lbs. of water at 120°F. The suspension was mixed for 10 minutes after which 476 lbs. of nitroglycerin were added. The suspension was again mixed for ten minutes after which a premixed suspension of 17.0 lbs. of ethyl centralite and 54.4 lbs. of lead beta-resorcylate was added. The slurry was mixed for 30 minutes after which the excess water was removed by centrifuging in a wringer to form a paste which was screened through a  $\frac{1}{4}$  inch by  $\frac{1}{4}$  inch mesh screen and dried until the moisture content was 8-12%. The paste was then blended, 17.0 lbs. of sodium barbiturate being added to the paste during the blending. The paste was then rolled on differential speed rolls at 210°F with a roll gap of 0.025 inch  $\pm$  0.005 inch at roller speeds of 22.5 and 15 rpm to obtain differential speed sheets. These sheets were then rolled on even speed rolls to form even speed sheets at 140°  $\pm$  10°F at a roll speed of 11 rpm and a roll gap of 0.035 inch  $\pm$  0.005 inch.

Sheets produced by the methods described above in Example I and Example II were prepared and tested for burning rate in the following manner. Strands,  $7 \times \frac{1}{8} \times \frac{1}{8}$  inches, were cut from the sheets and ignited by a hot wire in the closed bomb of a conventional strand burning apparatus at specified temperatures and pressures. The time required for the ignited strand to burn a specified length is used to calculate the strand burning rate of the propellant. The burning rates obtained

were set forth in the table below and compared to the conventional burning rates of the compositions described in the application which has been heretofore cited.

TABLE I

| BURNING RATES<br>CONVENTIONAL COMPOSITIONS |         |         |         |         |
|--------------------------------------------|---------|---------|---------|---------|
| Low Temp.                                  | SMU-101 | SMU-102 | SMU-118 | SMU-119 |
| Pressure*                                  |         |         |         |         |
| 400                                        | 0.158   | 0.133   | 0.233   | 0.224   |
| 600                                        | 0.158   | 0.156   | 0.274   | 0.263   |
| 800                                        | 0.078   | 0.168   | 0.302   | 0.292   |
| 900                                        | 0.086   | 0.168   | 0.323   | —       |
| 1000                                       | 0.087   | 0.166   | 0.337   | 0.304   |
| 1100                                       | 0.095   | 0.162   | 0.331   | —       |
| 1200                                       | 0.101   | 0.154   | 0.340   | 0.309   |
| 1400                                       | 0.114   | 0.151   | 0.328   | 0.292   |
| 1600                                       | 0.128   | 0.164   | 0.329   | 0.267   |
| 1800                                       | 0.142   | 0.178   | 0.303   | 0.234   |
| 2000                                       | 0.159   | 0.193   | 0.279   | 0.230   |
| Ambient Temp.                              | 70°F    | 70°F    | 70°F    | 70°F    |
| Pressure*                                  |         |         |         |         |
| 400                                        | 0.162   | 0.158   | 0.248   | 0.270   |
| 600                                        | 0.135   | 0.181   | 0.277   | 0.317   |
| 800                                        | 0.125   | 0.186   | 0.360   | 0.340   |
| 900                                        | 0.118   | 0.181   | 0.385   | —       |
| 1000                                       | 0.138   | 0.177   | 0.380   | 0.338   |
| 1100                                       | 0.142   | 0.180   | 0.383   | —       |
| 1200                                       | 0.151   | 0.181   | 0.386   | 0.324   |
| 1400                                       | 0.170   | 0.191   | 0.389   | 0.305   |
| 1600                                       | 0.180   | 0.208   | 0.357   | 0.292   |
| 1800                                       | 0.206   | 0.216   | 0.328   | 0.284   |
| 2000                                       | 0.204   | 0.230   | 0.298   | 0.301   |
| High Temp.                                 | 160°F   | 160°F   | 145°F   | 165°F   |

\*Pounds per square inch

A comparison of the data, set forth in Table 1, illustrates that the conventional smokeless double-base propellants compositions into which the lead resorcylate is incorporated are useful as propellants at entirely different temperatures and pressures. Further, burning rates, which were heretofore unobtainable with the conventional compositions available, are now achieved with compositions having lead resorcylate as an ingredient and therefore such compositions may be utilized

to advantage in the specialized propulsion systems in use today.

Further, propellant compositions, processed, in accordance with the procedures set forth in Examples I and II, were then rolled into 15 inch carpet rolls and extruded in a 15 inch press through a die approximately 4 inches in diameter. Thereafter, several 2 inch test motor grains were fabricated from these extrusions. The motor grains had the following dimensions, viz: (a) a length of 7.25 inches, (b) an outside diameter of 1.75 inches, and (c) an inside diameter of 0.6 inches. When the machined grains were fired in standard 2 inch rocket test motors, the attenuation of a beam of light by the exhaust gases was measured and compared to similar data which had been obtained for a conventional propellant at ambient temperature. This data is set forth in the Table below.

In view of the data given above, it is quite evident that the propellant produced in accordance with this invention gives rise to exhaust products having less smoke than conventional smokeless propellants. This was confirmed by visual observation of the firings on a closed circuit television screen and motion picture films of the static firing which shows that the propellant into which lead resorcylate is incorporated produces a cleaner exhaust than conventional smokeless propellants. Further, the pressure produced by the present propellants have ideal operating pressures within the range desired for the propulsion systems in use today.

This invention retains the synergistic effects taught in the above cited application while tailoring the burning rate and ideal operating pressure of the propellant to suit the conventional and special equipment in use today. This is basically accomplished by incorporating the lead salt of a resorcylate into a smokeless nitrocellulose double-base propellant already containing the sodium salt of a ureide.

Obviously, there are many modifications and variations which are possible in view of the above teachings. It is therefore to be understood that these modifications and variations are to be included within the scope of the appended claims.

I claim:

1. In a smokeless double-base propellant containing nitrocellulose and nitroglycerin, the improvement consisting of the incorporation in said propellant of the sodium salt of a ureide and a lead resorcylate to produce the synergistic effects of cleaner exhaust, a burning rate

TABLE II

|                                     | Conventional Propellant | Propellant<br>SMU-118 | Propellant<br>SMU-119 |
|-------------------------------------|-------------------------|-----------------------|-----------------------|
| Calculated<br>Flame Temp.<br>(°F)   | 2523                    | 2540                  |                       |
| Heat of<br>Explosion<br>cal/gm      | 700                     | 704                   |                       |
| Static Firing<br>Data               |                         |                       |                       |
| Pressure, psi                       | 710                     | 1268                  | 1048                  |
| Mass rate of<br>discharge<br>lb/sec | 0.340                   | 0.795                 | 0.792                 |
| Light Attenuation,<br>%             | 3.7                     | 2.81                  | 3.18                  |
| Specific Attenuation*               | 10.9                    | 3.53                  | 4.02                  |

\*Light attenuation divided by mass rate of discharge.

of over about 0.25 inches per second, and an operating pressure of over about 1000 pounds per square inch.

2. The composition of claim 1 wherein said lead resorcylate is lead alpha-resorcylate.

3. The composition of claim 1 wherein said lead resorcylate is lead beta-resorcylate.

4. The composition of claim 1 wherein said lead resorcylate is lead gamma-resorcylate.

5. The composition of claim 1 wherein said lead resorcylate is present in an amount between about 0.5 and 10.0 percent by weight.

6. The composition of claim 1 wherein said lead resorcylate is present in an amount of about 3.2 percent by weight.

7. The composition of claim 1 which contains sodium barbiturate and lead beta-resorcylate.

8. The composition of claim 1 which contains sodium barbitol and lead beta-resorcylate.

9. The composition of claim 2 wherein said lead alpha-resorcylate is present in an amount between about 0.5 and 10.0 percent by weight.

10. The composition of claim 2 wherein said lead alpha-resorcylate is present in an amount of about 3.2 percent by weight.

11. The composition of claim 3 wherein said lead

beta-resorcylate is present in an amount between about 0.5 and 10.0 percent by weight.

12. The composition of claim 3 wherein said lead beta-resorcylate is present in an amount of about 3.2 percent by weight.

13. The composition of claim 4 wherein said lead gamma-resorcylate is present in an amount between about 0.5 and 10.0 percent by weight.

14. The composition of claim 4 wherein said lead gamma-resorcylate is present in an amount of about 3.2 percent by weight.

15. The composition of claim 7 wherein said lead beta-resorcylate is present in an amount between about 0.5 and 10.0 percent by weight.

16. The composition of claim 7 wherein said lead beta-resorcylate is present in an amount of about 3.2 percent by weight.

17. The composition of claim 8 wherein said lead beta-resorcylate is present in an amount between about 0.5 and 10.0 percent by weight.

18. The composition of claim 8 wherein said lead beta-resorcylate is present in an amount of about 3.2 percent by weight.

\* \* \* \* \*